

# UNITED STATES PATENT OFFICE.

NICHOLAS CONLON, OF LAKE, ILLINOIS.

## TREATING CRUDE ANIMAL-HAIR.

SPECIFICATION forming part of Letters Patent No. 387,579, dated August 7, 1888.

Application filed March 1, 1886. Serial No. 193,692. (No specimens.)

*To all whom it may concern:*

Be it known that I, NICHOLAS CONLON, a citizen of the United States, residing at No. 802 Forty-third street, in the town of Lake, 5 county of Cook, and State of Illinois, have invented certain new and useful Improvements in the Process of Cleansing, Deodorizing, and Rendering Moth-Proof Crude Animal-Hair, more especially crude hog-hair, and preparing it economically and expeditiously for market; and I do hereby declare that the following is a full, clear, and exact description of the invention, which will enable others skilled in the business to which it belongs to make and 15 apply the same.

The process now generally followed consists in spreading out on the ground the crude hair as it comes from the scalding-tub, scraping-bench, and slaughter-house, and allowing the 20 impurities and foreign matter therein, consisting of the dirt, blood, cuticle, shreds of skin, flesh, and other animal matter, as far as may be, to disintegrate, decay, or dry up under the action of the elements, keeping it raked and turned over from time to time to 25 avoid the deterioration and destruction of the underlying hair by heating or otherwise, and when thus sufficiently dried and partly deodorized preparatory to shipping, sending it to the hair-factory to be cleansed, deodorized, and prepared for market. Under this 30 treatment the crude hair cannot be efficiently handled in winter, while during the year, by reason of the winds, much light hair is blown away, in addition to the loss from heating, &c., 35 thus materially lessening the quantity saved, as well as deteriorating its quality in color, strength, elasticity, and durability. The crude hair often remains six to eight months on the ground before it is in a fit condition to ship, 40 during which the effluvia arising from the putrefying and decaying animal matter contaminates the air for some distance around.

The object of my invention is by one continuous process to cleanse, deodorize, render moth-proof, improve the quality, and expeditiously prepare for market crude animal-hair, more especially crude hog-hair.

By my process I save all the hair as it comes 45 from the slaughter-house, and I cleanse, deodorize, and render it moth-proof at any sea-

son of the year without in any way injuring its elasticity, strength, or durability, and perform in a few days the work it now takes the elements and factory combined months to effect, while the sanitary benefit resulting from my treatment cannot be overestimated in and around populous cities.

To carry my invention into effect I first thoroughly wash the crude hair in water. I do not confine myself to any temperature, but prefer to use it at a temperature of 60° Fahrenheit. I next prepare a solution or compound of matter consisting of the following ingredients, combined in the proportions 65 stated, viz: two hundred (200) pounds pure water, four and one-half (4½) pounds quicklime, one and three-fourths (1¾) pound sal-soda, and one (1) pound sulphuric acid. I contemplate using any chemical equivalents of 70 quicklime, sal-soda, and sulphuric acid as substitutes therefor, whether such equivalents be simple or compound chemical equivalents. I prefer the above solution, but it may be varied. These ingredients should be thoroughly 75 mixed in a tub or vat, at the bottom of which there should be a coiled pipe or worm, through which steam can be passed for the purpose of boiling the compound.

I place the crude hair, after washing, in a 80 wire basket or crib made to fit into said tub or vat, and furnished with adjustable wire covers to keep the hair under the water-line while in process of cooking, and with like adjustable bottom for the purpose of protecting 85 it from contact with the worm or steam-coil, and for promptly emptying the basket when taken out of the vat and boiling compound. This basket or crib with its contents, by means of suitable machinery, I suspend in the com- 90 pound or solution above described in such manner as will completely cover the crude hair with the compound. I do not confine myself to any special contrivance, but prefer the above.

Having immersed the crude hair 95 in the compound, as above described, I turn on the steam and bring the solution to 212° Fahrenheit, keeping it at that temperature until such time as the hair is properly cooked, varying from three to five hours. In cooking, 100 the steam may be allowed to run from the coil or worm in and through the solution by means

of small perforations in the coil or worm; or it may be taken through the coil or worm without contact with the compound. I do not confine myself to either process, but prefer the latter. Neither do I confine myself to immersing the hair in the compound before applying steam, as the hair may be immersed at any temperature under 212° Fahrenheit with satisfactory results. I prefer, however, to use

10 as above described.

I ascertain by examination from time to time when the hair is sufficiently cooked. The changing of the shreds of cuticle, flesh, &c., into a gelatinous substance that can be easily removed by rubbing is generally a sufficient indication. When cooked sufficiently, I hoist the wire basket and its contents, above described, by the aid of suitable machinery, out of the tub or vat and the boiling compound there-  
15 in and carry it to a second tub or vat filled with warm water at a temperature between 150° and 180° Fahrenheit, into which I quickly dump the contents of the wire basket for wash-  
ing, &c.

20 Under the process of cooking, the foreign matter in the crude hair, consisting of the shreds of cuticle, flesh, &c., becomes of a gelatinous character, and by rubbing, teasing, and washing is easily detached and removed from  
25 the hair. With the object of attaining this result, when removing the hair from the sec-  
ond vat or tub, I rub, tease, and wash it free from all gelatinous and extraneous matter by  
30 the use of suitable machinery for that purpose,  
35 and deliver the hair, after being so treated, thoroughly cleansed, and partly deodorized and ready for deodorizing and moth-proofing.

I do not confine myself to any special class or kind of machinery for the rubbing, teasing, and washing of the hair; but I prefer to use  
40 that caveat on July 11, 1885, by Francis Murphy, of Chicago, Illinois, for washing un-  
manufactured fibrine material.

Having thus cleansed the hair, I then im-  
45 merse it in a vat or tub containing a solution or composition of matter consisting of the fol-  
lowing ingredients combined in the propor-  
tions stated, viz: two hundred (200) gallons  
50 water, one (1) gallon of a solution of the black oxide of manganese and sulphuric acid pre-  
pared as follows, viz: To one hundred and  
sixty pounds of sulphuric acid, standard  
strength, I add thirteen and one-half pounds of  
55 the black oxide of manganese and allow it to  
remain in solution from twelve to fifteen days,

stirring the compound occasionally, after which I reduce it with water to 85° Twaddle's hydrometer, when it is ready for use in the proportions above given. I boil the hair in the above solution from ten to thirty minutes  
60 by means of a steam-coil in the bottom of the vat or tub, as hereinbefore described; but I do not allow the steam to escape in the solution. When sufficiently cooked, it becomes thor-  
oughly deodorized and moth-proof, and may  
65 be dyed, curled, and dried for market.

I prefer the above solution and treatment  
for the purpose of deodorizing and rendering  
the hair moth-proof; but the proportions of  
the ingredients in the solution may be varied  
70 and the time for cooking increased or diminished,  
and hence I do not confine myself to either the proportions named, or time specified,  
nor to any particular style of tubs, vats,  
or machinery.

Having fully described my invention, what I  
desire to claim and secure by Letters Patent  
is—

The process hereinbefore described of cleans-  
ing, deodorizing, and rendering moth-proof  
80 crude animal-hair, more particularly crude  
hog-hair, which consists in washing said hair  
to remove the blood and extraneous dirt, &c.,  
and cooking the hair in a compound or solu-  
tion of water, quicklime, sal-soda, and sul-  
phuric acid for the purpose of changing the  
85 cuticle and shreds of flesh, &c., into a gelati-  
nous substance, and thereby rendering its  
separation from the hair the more easily  
effected, afterward rubbing, teasing, and wash-  
90 ing the said hair to remove the gelatinous  
matter and complete the cleansing process,  
and again cooking the same in a compound or  
solution of water combined with a solution of  
sulphuric acid and black oxide of manganese  
95 for the purpose of further deodorizing and  
rendering it moth-proof, thus preparing it for  
dyeing, curling, and drying in one continuous  
expeditious and economical process, substan-  
tially as and for the purposes hereinbefore de-  
scribed.

In testimony whereof I have signed my name,  
in the presence of William Kirby and Francis  
W. McNally, subscribing witnesses, this 23d  
day of February, A. D. 1886.

NICHOLAS CONLON.

In presence of--

WILLIAM KIRBY,  
F. W. MCNALLY.